

Nov. 16, 1965

A. W. SPEARS ETAL

3,217,719

CIGARETTE FILTERS CONTAINING SELECTIVE ADSORBENTS

Filed April 16, 1962



INVENTORS:  
ALEXANDER W. SPEARS  
WILLIAM E. ROUTH  
CHASE W. LASSITER  
JIMMY H. BELL  
BY

*Brown, Brey, Gross and Dorfman*  
THEIR ATTORNEYS

3,217,719

CIGARETTE FILTERS CONTAINING SELECTIVE  
ADSORBENTS

Alexander W. Spears, William E. Routh, Chase W. Lassiter, and Jimmy H. Bell, all of Greensboro, N.C., assignors to P. Lorillard Company, New York, N.Y., a corporation of New York

Filed Apr. 16, 1962, Ser. No. 188,281  
6 Claims. (Cl. 131—208)

This invention relates to a new tobacco smoke filter which selectively removes certain products of combustion in tobacco smoke, and particularly to cigarette filters having a chemical complexing agent to selectively remove phenol and phenolic compounds in tobacco smoke.

According to the present invention, it has been found that a tobacco smoke filter containing a polymeric compound having the property of forming a complex with the phenol and phenolic compounds has a greatly improved efficiency for removing phenols and phenolic compounds from tobacco smoke.

Compounds which have been found to be particularly useful in this respect are polymers and copolymers of N-vinyl-5-methyl-2-oxazolidinone. In the copolymers, the active moiety is the oxazolidinone unit having the structural formula:



Polymers or copolymers containing from 25 to 100% of the N-vinyl-5-methyl-2-oxazolidinone unit have useful complexing activity. Monomers suitable for copolymerization with N-vinyl-5-methyl-2-oxazolidinone include, but are not limited to, vinyl acetate. Other useful monomers would be those which contain the vinyl group (styrene, vinyl acetate, etc.).

The molecular weight of the complex-forming compounds is dependent on the specific material used. In selecting a suitable molecular weight, the vapor pressure of the complex-forming compound should be sufficiently low that it will remain in the filter during storage, and will not volatilize during the smoking of the cigarette. The vapor pressure of such complex-forming compounds should be from 0 mm. up to 40 mm. Hg at 25° C., however, the preferred range is between 0 mm. and 1 mm. Hg at 25° C.

According to the present invention, the complex-forming compounds are incorporated in a conventional tobacco smoke filter, usually made of cellulose or substituted cellulose fibers. However, the filter may be composed of natural fibers, mineral fibers and other synthetic fibers such as nylon, polypropylene and polyethylene. Mixtures of synthetic, mineral and natural fibers are also suitable. By manufacturing methods well known in the art, the fibers are formed into a compact plug having a plurality of tortuous passages to trap small diameter solid and liquid par-

ticulate matter present in the tobacco smoke. The filter fiber provides support for the complex-forming compounds of the present invention, and accordingly no particular form or type of fiber material is required for the successful practice of this invention.

5 A typical filter-cigarette is illustrated in FIG. 1. This comprises a plug of shredded tobacco 1 and, superimposed thereon, a tip comprising a plug of compact, fibrous base material 3. The filter tip and tobacco are joined in a unitary structure by a suitable wrapping paper 2. In the practice of the present invention, the fibrous base material 3 is impregnated with polymers or copolymers of N-vinyl-5-methyl-2-oxazolidinone as described above. Depending on the method of impregnation, the selective adsorbents 10 may form a thin film over the individual strands of fibrous material, or may be absorbed into the fibrous material, or as illustrated it may be in the form of a powder 4 supported by the fibrous base material 3.

The complex-forming compounds according to the present invention may be applied to the filter fibers before formation of the plug, and the amount of complex-forming compound may range from 0.01% to 100% by weight of the filter depending upon the manner in which the complex-forming compound is used. Some complex-forming compounds may be incorporated into the filter as a solid powder. In that case, complex-forming compound is preferably present in an amount between 5% and 25% by weight of fiber. In other cases the complex-forming compounds are more conveniently incorporated 15 into the filter with the aid of a solvent, a compatible non-toxic plasticizer or both. Where the solvent technique is used, the complex-forming compound may be present in an amount between 0.01% and 25% by weight of fiber, the optimum range being between 0.3% and 2% by weight of fiber.

20 Suitable plasticizers are glyceryl triacetate, triethyl citrate, acetyl triethyl citrate and alkyl phthalates. The plasticizers should be present in amounts up to 20% by weight.

In still another method the complex-forming compounds 25 may be formed into a filter by fusion, sintering or other direct fabrication method. In such case, the entire filter plug is composed of the complex-forming compound.

30 Cigarette filters, according to the present invention, are illustrated by the following examples. As a basis of comparison, two types of filters using chemically inert materials are used as standards, namely a typical commercial filter of cellulose acetate and a filter comprised of cellulose acetate into which has been incorporated a powder which is inert with respect to phenol. The cigarettes were 35 "machine smoked" and the products passing through the filter were collected and analyzed. The physical and filtration properties of these filters are given in Table 1. The selectivity of the cellulose acetate filter is probably due to an association complex between phenol and the oxygen atoms of the acetyl group.

40 The terms "filter efficiency" and "phenol filter efficiency" used in the following table and examples refer to the percentages of particulate matter and of phenol and phenolic compounds removed from the tobacco smoke.

TABLE 1

| Filter Material                             | Length, mm. | Plasticizer            | Filter Weight | Denier of Fiber | Total Denier | Plug Draw | Total Filtration Efficiency, percent | Filtration Efficiency of Phenol, percent | Selective Removal of Phenol, percent |
|---------------------------------------------|-------------|------------------------|---------------|-----------------|--------------|-----------|--------------------------------------|------------------------------------------|--------------------------------------|
| Polyethylene-----                           | 17          | -----                  | -----         | <1              | 19,000       | .29       | 69.0                                 | 61.5                                     | -7.5                                 |
| Propylene-----                              | 17          | -----                  | -----         | 3               | 55,000       | .39       | 50.0                                 | 54.5                                     | 4.5                                  |
| Cellulose acetate-----                      | 17          | 6% glyceryl triacetate | -----         | 3.2             | 55,000       | .48       | 47.0                                 | 71.5                                     | 24.5                                 |
| Cellulose acetate and 15% cellulose powder. | 17          | do                     | -----         | 3.2             | 55,000       | .36       | 56.0                                 | 81.5                                     | 25.5                                 |

*Example I*

In accordance with this example, a dry powdered polymeric material is mixed with a filter fiber. The fiber-powder mixture is then formed into a cigarette filter plug by conventional techniques. Table 2 shows the filtering efficiency obtained with two such filters.

TABLE 2.—FILTERS CONTAINING POWDERED COMPLEX-FORMING COMPOUND

| Complex-forming Compound                                     | Wt. Percent on Fiber | Denier of Fiber | Total Denier | Length, mm. | Plug Draw | Total Filter Efficiency, Percent | Phenol Filter Efficiency, Percent |
|--------------------------------------------------------------|----------------------|-----------------|--------------|-------------|-----------|----------------------------------|-----------------------------------|
| 40 mesh poly [N-vinyl-5-methyl-2-oxazolidinone] <sup>1</sup> | 22                   | 3.2             | 55,000       | 17          | 0.43      | 49                               | 84                                |

<sup>1</sup> Commercially available from the Dow Chemical Corporation under the trade name "Devlex 130", and described in the "Dow Chemical Corporation Technical Bulletin Devlex 130" issued August 1960. The polymer used has a molecular weight of about 150,000.

*Example II*

A second method of incorporating the complex-forming compound into a cigarette filter is by use of a solvent technique. An exemplary solution consists of a copolymer of N-vinyl-5-methyl-2-oxazolidinone and vinyl acetate (in which the monomeric units are present in approximately equal mol ratios), ethanol and glycerol triacetate in the weight ratio 1:2:7, respectively. The solution of polymer, plasticizer and solvent was mixed with the cellulose acetate fibers at a concentration of 6% by weight. The filter fiber used had a denier of 3.2. Filter plugs were formed of the fibers. The filter plugs had a total denier of 55,000, a length of 17 mm., and a plug draw of 0.49. The total filter efficiency was 49% while the phenol filter efficiency was 85.5%.

The copolymer used in this example is commercially available from the Dow Chemical Company under the trade name Devlex A515, and is described in "Dow Chemical Corporation Bulletin, Devlex A515" issued August 1960.

The various filters set forth in the preceding examples have been described for exemplary purposes only, and it will be understood that the invention is not limited thereto except within the scope of the following claims.

We claim:

1. A filter element for filter tip cigarettes consisting essentially of a plug of a base material having a plurality of passages for trapping particulate matter in tobacco smoke and selected from the group consisting of cellulose, substituted cellulose, nylon, polypropylene and polyethylene fibers, said element containing a polymeric compound selected from the group consisting of polymers and copolymers containing the N-vinyl-5-methyl-2-oxazolidinone unit.

2. A filter element for filter tip cigarettes consisting essentially of a plug of a base material having a plurality of passages for trapping particulate matter in tobacco smoke and selected from the group consisting of cellulose, substituted cellulose, nylon, polypropylene and

4  
polyethylene fibers, said element containing a polymeric compound selected from the group consisting of polymers and copolymers containing the N-vinyl-5-methyl-2-oxazolidinone unit, said polymeric compound having a vapor pressure of 0 mm. to 40 mm. Hg at 25° C.

5. A filter element for filter tip cigarettes according to

claim 2 wherein said polymeric compound has a vapor pressure of 0 mm. and 1 mm. Hg at 25° C.

20. A filter element for filter tip cigarettes consisting essentially of a plug of a base material having a plurality of passages for trapping particulate matter in tobacco smoke and selected from the group consisting of cellulose, substituted cellulose, nylon, polypropylene and polyethylene fibers, said element containing a polymeric compound selected from the group consisting of polymers and copolymers containing the N-vinyl-5-methyl-2-oxazolidinone unit, said polymeric compounds having a vapor pressure of 0 mm. to 40 mm. Hg at 25° C. and being present in an amount from 0.01% to 100% by weight of said filter.

25. A filter element for filter tip cigarettes according to claim 4 wherein said polymeric compound is poly[N-vinyl-5-methyl-2-oxazolidinone].

30. A filter element for filter tip cigarettes according to claim 4 wherein said polymeric compound is a copolymer containing from 25% to 100% of the N-vinyl-5-methyl-2-oxazolidinone unit.

## References Cited by the Examiner

## UNITED STATES PATENTS

|           |        |                   |       |          |
|-----------|--------|-------------------|-------|----------|
| 2,707,959 | 3/1955 | Shelanski         | ----- | 131—10   |
| 2,839,065 | 6/1958 | Milton            | ----- | 131—10   |
| 2,902,998 | 9/1959 | Durandeau         | ----- | 131—9    |
| 2,933,460 | 4/1960 | Richter et al.    | ----- | 131—10   |
| 2,941,906 | 6/1960 | Haden             | ----- | 131—17   |
| 2,941,907 | 6/1960 | Tousignant et al. | ----- | 131—17   |
| 2,946,772 | 7/1960 | Walles et al.     | ----- | 260—88.3 |
| 2,946,773 | 7/1960 | Walles et al.     | ----- | 260—88.3 |
| 2,948,656 | 8/1960 | Tousignant et al. | ----- | 260—88.3 |

## FOREIGN PATENTS

55. 760,772 11/1956 Great Britain.

ABRAHAM G. STONE, Primary Examiner.

MELVIN D. REIN, Examiner.